

Patented Feb. 2, 1926.

1,571,382

# UNITED STATES PATENT OFFICE.

TORSTEN GEORG STIG AND JOSEF EINAR LEONARD STIG, OF ODDA, NORWAY.

METHOD OF PRODUCTION OF ALLOYED STEEL AND IRON WITH CHROMIUM,  
MANGANESE, ETC.

No Drawing.

Application filed March 21, 1924. Serial No. 700,945.

To all whom it may concern:

Be it known that we, TORSTEN GEORG STIG and JOSEF EINAR LEONARD STIG, both subjects of the King of Sweden, and both residing at Odda, Hardanger, Norway, have invented a certain new and useful Method of Production of Alloyed Steel and Iron with Chromium, Manganese, &c., of which the following is a specification.

10 In the production of some alloyed steel and iron, where a relative high amount of the added alloy metal is desired, while the amount of carbon is to be kept rather low, it is necessary to use an alloy with a very 15 low amount of carbon, which is rather expensive.

As a rule the amount of silicon ought to be low, but on the other hand it is easier to remove the carbon from an alloy with 20 a high amount of silicon than from an alloy low in silicon, for instance by bessemerizing, because practically all carbon can be oxidized in a few minutes. If the blowing with oxidizing gases is continued long 25 enough the same result may be attained with the silicon, but there is the risk in this case that the metal will absorb so large a quantity of petroleum that its quality is affected.

According to the present invention the 30 following process is used:

The bessemerizing is interrupted at the point when the carbon is oxidized down to the amount desired, while the rest of the silicon is afterwards removed by 35 metal oxides. The incompletely bessemerized metal is pulverized and mixed very carefully with a suitable quantity of pulverized metal oxides, which by sufficiently high temperature oxidizes the silicon, while 40 the oxides are reduced to metal. This reaction proceeds easiest if the mixture in the form of briquettes is added to the iron or steel directly before the discharge. Because the reaction is exothermic, the loss of heat

45 will be less than if the resulting alloy with a low amount of silicon is used and this heat evolution can still be increased by the addition of the known mixture of pulverized aluminum and metal oxides.

Having now described our invention, what we claim as new and desire to secure by Letters Patent is:—

1. Process of producing alloyed steel and iron which consists in bessemerizing an alloy until the carbon content is decreased to the desired degree but not lower than that required to retain a sufficient amount of silicon to avoid the formation of nitrides, pulverizing the product, mixing the pulverized product with a suitable quantity of 55 pulverized metal oxides to oxidize the remaining silicon, introducing the mixture into melted iron or steel to form an alloy, and discharging the alloy thus formed.

2. Process of producing alloyed steel and iron with chromium which consists in bessemerizing an alloy until the carbon content is decreased to the desired degree but not lower than that required to retain a sufficient amount of silicon to avoid the 70 formation of nitrides, pulverizing the product, mixing the pulverized product with a suitable quantity of pulverized metal oxides to oxidize the remaining silicon, briquetting the mixture, introducing the briquettes 75 into melted iron or steel to form an alloy and discharging the alloy thus formed.

3. Process of producing alloyed steel and iron with chromium which consists in bessemerizing an alloy until the carbon content is decreased to the desired degree but not lower than that required to obtain a sufficient amount of silicon to avoid the formation of nitrides, pulverizing the product, mixing the pulverized product with 80 a suitable quantity of pulverized metal oxides to oxidize the remaining silicon, briquetting the mixture, introducing the briquettes into melted iron or steel, with the addition also of the requisite quantity 85 of pulverized aluminum and metal oxides to obtain the required temperature, and discharging the alloy thus formed.

In testimony whereof we have signed our names to this specification.

TORSTEN GEORG STIG.  
JOSEF EINAR LEONARD STIG.